

- [54] **SOLID PROPELLANT FORMULATION  
CONTINUING FLUORO-AMINO  
COMPOUNDS AND POLYMERS**
- [75] Inventors: **Herman Bieber, Kenilworth;  
Lawrence Spenadel, Fanwood, both  
of N.J.**
- [73] Assignee: **Exxon Research & Engineering Co.,  
Linden, N.J.**
- [22] Filed: **May 17, 1961**
- [21] Appl. No.: **111,131**
- Related U.S. Application Data**
- [63] Continuation-in-part of Ser. No. 77,470, Dec. 21,  
1960, Pat. No. 3,535,173.
- [52] U.S. Cl. .... **149/19.3, 149/20, 149/19.9,  
149/22, 149/36, 149/75, 149/89**
- [51] Int. Cl. .... **C06d 5/06**
- [58] Field of Search .... **149/19, 20, 22, 36, 44  
149/89, 75, 71**

- [56] **References Cited**  
UNITED STATES PATENTS  
3,369,943 2/1968 Longwell et al. .... 149/18

3,425,922 2/1969 Guthrie ..... 149/19 X

Primary Examiner—Benjamin R. Padgett  
Attorney, Agent, or Firm—Henry Berk

#### EXEMPLARY CLAIM

1. A high-energy composite which on ignition burns at a controlled rate at a specific impulse in the range of 260 to 300 seconds, comprising 2 to 15 wt. percent boron, 5 to 25 wt. percent of a CNF<sub>2</sub> oxidizer selected from the group consisting of tetrakis (difluoramino) butane and tetrakis (difluoramino) tetrahydrofuran, 40 to 60 wt. percent of an oxygen oxidizer selected from the group consisting of nitronium perchlorate, hydrazinium nitroformate, hexanitroethane and ammonium perchlorate, and 5 to 30 wt. percent of a solid polymeric binder having the composition of polybutadiene (N<sub>2</sub>F<sub>4</sub>) adducts represented by the recurring unit composition [C<sub>4</sub>H<sub>6</sub>(NF<sub>2</sub>)<sub>y</sub>] in which y represents 1.3 to 2 NF<sub>2</sub> groups per recurring unit, the boron being in a 1:1 atomic ratio to fluorine in the composite to form BOF as a main combustion product.

5 Claims, No Drawings

SOLID PROPELLANT FORMULATION  
CONTINUING FLUORO-AMINO COMPOUNDS  
AND POLYMERS

This application is a continuation-in-part of U.S. application Ser. No. 77,470, filed Dec. 21, 1960 by L. Spenadel and H. Bieber, now U.S. Pat. no. 3,535,173, and which discloses the use of liquid compounds having a high proportion of  $\text{NF}_2/\text{C}$  groups to plasticize solid polymeric binders containing  $\text{NF}_2$  groups to form plastiols. These solid and liquid compounds are termed  $\text{CNF}_2$  compounds for brevity, indicating that they contain  $\text{NF}_2$  groups linked to carbon atoms.

This invention relates to solid propellants formulated from a powdered boron fuel, a solid oxygen-oxidizer, a high-energy binder containing  $\text{NF}_2$  groups, and a plasticizer containing  $\text{NF}_2$  groups, these ingredients being proportioned to obtain satisfactory burning rates at high impulse levels.

Work on combustion of propellants containing the solid and liquid compounds of high  $\text{NF}_2/\text{C}$  contents has shown that these propellants have excessively fast burning rates, especially those containing high amounts of the  $\text{CNF}_2$  liquid plasticizers. For example, a propellant containing boron, ammonium perchlorate as oxygen-oxidizer,  $\text{CNF}_2$  polymer as binder with the liquid  $\text{C}_3\text{H}_5(\text{NF}_2)_3$  as plasticizer has a burning rate of 15 inches per second at 500 psi. when these ingredients are compounded to make the propellant's  $\text{NF}_2$  content 45 wt. percent. The impulse (Isp) of this propellant is only 260.

Studies show that propellant compositions having a high  $\text{NF}_2$  content have high burning rate when balanced to form  $\text{BF}_3$  or  $\text{HF}$  (with no B present). Such compositions can have Isp values higher than 260, but not at realistic burning rates. At the high burning rates there is a tendency to detonation. In such systems the oxygen-supplying oxidizer is present in a proportion to burn the carbon, e.g., to form  $\text{CO}$ . The boron is reacted with fluorine to form  $\text{BF}_3$ .  $\text{H}$  is either burned to  $\text{HF}$  or discharged as  $\text{H}_2$ .

In accordance with the present invention, the propellants containing boron, oxygen-oxidizer, and  $\text{CNF}_2$  compounds are balanced to form  $\text{BOF}$ . This enables achievement of Isp values in the range of about 265 to 300 with desirable burning rates of about 0.5 to 2.0 inches per second.

There is a marked advantage for the system balanced to  $\text{BOF}$  formation when compared to those balanced to  $\text{BF}_3$  formation on a constant Isp basis (thrust in pounds force per second per pound of propellant).

Basically, to obtain a propellant balanced for  $\text{BOF}$  formation, less  $\text{CNF}_2$  liquid is required as fluorine-oxidizer and plasticizer and the resultant propellant has an  $\text{NF}_2$  content preferably less than 30 wt. percent. Enough oxygen-oxidizer is used to supply  $\text{O}$  for  $\text{BOF}$  and to burn carbon to  $\text{CO}$ . The binder and  $\text{CNF}_2$  liquid are used in a proportion to supply  $\text{F}$  for  $\text{BOF}$ . The binder is used in sufficient amount to give structural strength of the solid propellant grain, e.g., usually 10 to 30 wt. percent of the composite.

The  $\text{CNF}_2$  solids and liquids are recent in their development. That is why burning rate effects of these materials compounded with fuels and other oxidizers have not been understood fully hitherto.

In a propulsion system, thrust is the reaction force produced by expelling particles of high velocity from a

combustion zone through a nozzle opening, the particles being gaseous, solid, liquid or even bundles of energy. In general, these particles are collectively termed "gas" or gaseous working fluid.

5 The specific impulse (Isp) is a measure of thrust and varies with temperature in the combustion chamber in which the propellant components of fuel and oxidizer undergo combustion. It is expressed usually as in terms of seconds.

10 Thrust of a system lasts only so long as working fluid is produced for expulsion and does not depend on total amount or density of propellant material. Therefore, another useful measure of performance is the relative boost velocity which is a function of density and of specific impulse of a propellant. The relative boost velocity (RBV) is evaluated with reference to a standard propellant.

In earlier studies, burning rates of propellants containing a  $\text{CNF}_2$  binder with a solid oxidizer such as per-

20 chlorate or nitroformate were found to rise rapidly with increased  $\text{CNF}_2$  liquid plasticizer added. These systems were balanced to form  $\text{HF}$  gas product. Next, it was found that boron powder could be added to such system in proportions to form  $\text{BF}_3$  or  $\text{BOF}$  combustion

25 products. The  $\text{BOF}$  system was then found to have a 30 to 50 percent faster burning rate than the  $\text{HF}$  or  $\text{BF}_3$  forming systems at the same  $\text{NF}_2$  level. However, the  $\text{BOF}$  system has an Isp above 270 at a 20 to 28 percent  $\text{NF}_2$  level, whereas the  $\text{HF}$  and  $\text{BF}_3$  systems have an Isp

30 in the range of 220 to 250 at this  $\text{NF}_2$  level. In the 265 to 300 specific impulse range the  $\text{HF}/\text{BF}_3$  systems are characterized by extremely rapid and unstable burning. The  $\text{HF}/\text{BF}_3$  systems have to contain 35 to 50 percent  $\text{NF}_2$  to obtain this higher impulse. Thus, the  $\text{BOF}$ -

35 forming systems were found to be preferred for high impulse and controlled burning. Since one might expect that burning rates increase with increasing energy content (higher Isp), the achievement of low burning rates at the 270 + Isp level (by formulating to  $\text{BOF}$ ) is quite surprising and novel.

Formulation of propellants containing  $\text{CNF}_2$  compounds with oxygen oxidizers and boron-supplying fuel to produce  $\text{BOF}$  rather than  $\text{BF}_3$  and  $\text{HF}$  is advantageous for better boost performance as well as for better

45 burning rate and higher Isp. The addition of boron increases density, which helps the boost velocity.

Whereas in fluorine oxidizing systems balanced to  $\text{HF}/\text{BF}_3$ , the boron is added to combine with fluorine in excess of the hydrogen, in the present disclosed systems of improved performance the fluorine available for reaction is lowered as the proportion of boron and oxygen from the oxygen oxidizer is increased.

The solid propellants or hot gas-generating composites of interest generally contain fuel constituents such as carbon hydrogen, and boron, fluorine oxidizing constituents in the  $\text{CNF}_2$  ingredients and oxygen oxidizing constituents in ingredients containing nitro groups, perchlorate groups, or both nitro and perchlorate groups.

50 The carbon and hydrogen constituents may come from a hydrocarbon moiety of the oxidizer and from a binder ingredient which may also contain  $\text{CNF}_2$ , nitro groups or both. The fuel, oxidizer, and binder ingredients may be intimately mixed and cast or otherwise shaped into a solid mass, called a grain, which is cemented or attached to a rocket case in its combustion chamber.

55 60 65 For testing purposes two types of systems were selected, one with a normal oxygen oxidizer, hydrazinium

nitroformate, the other with a more energetic oxygen oxidizer, hexanitroethane. The systems compared were:

TABLE 1

|                   |                                                        |                                                                               |
|-------------------|--------------------------------------------------------|-------------------------------------------------------------------------------|
| Fuel              | -boron                                                 | B                                                                             |
| Fluorine Oxidizer | -tetrakis (NF <sub>2</sub> ) butane                    | C <sub>4</sub> H <sub>6</sub> (NF <sub>2</sub> ) <sub>4</sub>                 |
| Oxygen Oxidizer   | -hydrazinium nitro-                                    | N <sub>2</sub> H <sub>5</sub> C(NO <sub>2</sub> ) <sub>3</sub>                |
|                   | formate                                                |                                                                               |
| Binder            | hexanitroethane                                        | C <sub>2</sub> (NO <sub>2</sub> ) <sub>6</sub>                                |
|                   | -polybutadiene (N <sub>2</sub> F <sub>4</sub> ) adduct | [C <sub>4</sub> H <sub>6</sub> (NF <sub>2</sub> ) <sub>2</sub> ] <sub>x</sub> |

The high NF<sub>2</sub> level formulations contained 30+ wt. percent NF<sub>2</sub>. The low NF<sub>2</sub> level formulations contained less than 30 wt. percent NF<sub>2</sub>. Observations were made on the effects of varying proportions of binder and oxygen oxidizer.

Increasing the boron content in the NF<sub>2</sub>-rich systems to form more BF<sub>3</sub> instead of HF as products of combustion lowers the impulse of the hot system containing C<sub>2</sub>(NO<sub>2</sub>)<sub>6</sub> as oxygen oxidizer but helps the impulse of the cool system containing N<sub>2</sub>H<sub>5</sub>C (NO<sub>2</sub>)<sub>3</sub> as oxygen oxidizer to a small extent.

| Burning Rate, In./Sec. at 500 psi | Isp, Sec.                    |             |
|-----------------------------------|------------------------------|-------------|
|                                   | BF <sub>3</sub> , HF Systems | BOF Systems |
| 0.50                              | 210                          | 240         |
| 0.75                              | 225                          | 260         |
| 1.0                               | 235                          | 275         |
| 2.5                               | 250                          | 286         |
| 00                                | 286                          | —           |

The systems formulated to contain less than 30 wt. percent NF<sub>2</sub> and to form H<sub>2</sub>-BOF products of combustion have higher impulses than those forcing HF+BF<sub>3</sub> or H<sub>2</sub>+BF<sub>3</sub> combustion products even with increasing proportions of binder. Added binder in proportions of about 10 to 30 wt. percent results in less dissociation of the propellant particularly with a sufficiently low proportion of boron, e.g., 2 to 10 wt. percent. The high NF<sub>2</sub> level systems have to contain more boron, are much hotter, and more dissociated.

The low NF<sub>2</sub> level system which forms BOF combustion product has a distinctly higher boost velocity compared to the other systems throughout variations in proportions of binder from 0 to 30 wt. percent.

In the preferred formulations containing B as fuel the atomic ratio of B/F in the ingredients and products is 1:1. The O/C ratio is generally about 2:1 or in the range of 1.8:1 to 2.8:1 since O is needed to form BOF as well as to form CO.

Powered boron is preferably used as the fuel ingredient to form the BOF combustion product. However, other ingredients that supply boron may be used, e.g., hydrazine bis borane, (N<sub>2</sub>H<sub>4</sub>(BH<sub>3</sub>)<sub>2</sub>) denoted by the abbreviation HBB or related boranes.

Among other potent fluorine oxidizers are compounds such as tetrakis (NF<sub>2</sub>) tetrahydrofuran and other acyclic or cyclic compounds having at least 1 NF<sub>2</sub> group per carbon atom, generally containing about three to six carbon atoms per molecule and preferably four to six carbon atoms per molecule. These compounds are beneficial in raising the Isp and in plasticizing potent binders which also contain NF<sub>2</sub> groups and/or nitro groups.

Among other potent oxygen oxidizers are bis (trinitroethyl) nitramine, nitroform, nitronium perchlorate, ammonium perchlorate, hydrazinium perchlorate, etc. Some of these are very reactive and have to be encapsulated in a compatible material such as aluminum or suitable resin. Generally, the oxygen oxidizers are solids and of relatively high density, e.g., about 1.6 to 2.2 g/cc.

The preferred binders are also energy suppliers in containing NF<sub>2</sub>, NO<sub>2</sub>, or both kinds of groups. The polybutadiene-N<sub>2</sub>F<sub>4</sub> adducts suitable as binders are represented by the formulae [C<sub>4</sub>H<sub>6</sub>(NF<sub>2</sub>)<sub>y</sub>]<sub>x</sub> or [C<sub>4</sub>H<sub>6</sub>(NF<sub>2</sub>)<sub>y</sub>]<sub>x</sub> in which y represents about 1.3 to 2 and x is the number indicating the number of recurring units. Other binders may be made to contain more or fewer NF<sub>2</sub> groups. Other high energy polymers are represented by polynitrourethane, polyvinyl furoate-N<sub>2</sub>F<sub>4</sub> adducts, nitrocellulose, etc. For balancing the compositions, lower energy polymers may be used in minor amounts, e.g., saturated or synthetic rubbers denoted generally by CH<sub>2</sub>)<sub>x</sub>. To achieve high impulse ratings in the range of 270 to 300, the high energy binder is preferably used in a proportion of about 10 to 30 wt. percent. Enough of the binder is employed to obtain the

desired cohesion of the mixed ingredients into a solid or plastisol mixture that hardens to a solid even with a liquid CNF<sub>2</sub> oxidizer-plasticizer admixed.

In preparing solid propellant grains from ingredients that contain the necessary fuel and oxidizing constituents, it is important to use methods that are safe and permit ease of handling.

The plastiols are mixtures of solid and liquid ingredients having adequately safe capabilities and which under conditions of mixing form a fluid or semi-fluid mass that becomes transformed into a solid gel having minimum rubbery properties. The rubbery mass obtained should have a tensile strength above 20 pounds per square inch and an elongation of over 10 percent, as minimum requirements of stiffness and elasticity.

After mixing the solid and liquid ingredients, the mixture can be cast or molded, then set by curing. The mixing, handling and curing may be carried out at moderate temperatures of about 20° to 60°C.

If the gel or plastisol is on the soft side, various reinforcing fibrous materials may be admixed, e.g., aluminum wool, or fibers of polymers or of other fuel ingredients for adding rigidity. Stiffness is imparted by increasing the proportion of binder.

In general the mixtures contain the ingredients in the following proportions:

| Component                 | Broad Range, Wt. % | Preferred Wt. % |
|---------------------------|--------------------|-----------------|
| CNF <sub>2</sub> Oxidizer | 5 to 25            | 5 to 20         |
| Boron                     | 2 to 15            | 5 to 15         |
| Oxygen Oxidizer           | 40 to 60           | 40 to 60        |
| Binder                    | 5 to 30            | 15 to 25        |

Examples of propellant compositions which produce BOF as the main F-containing product are the following:

TABLE 2

|      | COMPOSITION          | WT. % | DENSITY<br>G./CC. | ISP | RBV   | MAIN<br>PRODUCTS |
|------|----------------------|-------|-------------------|-----|-------|------------------|
| I    | $C_4H_6(NF_2)_4$     | 10.24 | 1.85              | 289 | 1.1   | BOF              |
|      | B                    | 11.59 |                   |     |       | CO               |
| II   | $NO_2ClO_4$          | 48.17 | 1.74              | 292 | 1.07  | HCl              |
|      | $[C_4H_6(NF_2)_2]_x$ | 30.00 |                   |     |       | $H_2+N_2$        |
| III  | $C_4H_6(NF_2)_4$     | 21.49 | 1.71              | 287 | 1.05  | BOF              |
|      | B                    | 11.20 |                   |     |       | CO               |
| IV   | $C_2(NO_2)_6$        | 52.30 | 1.76              | 278 | 1.03  | $H_2$            |
|      | $[C_4H_6(NF_2)_2]_x$ | 15.00 |                   |     |       | $N_2$            |
| V    | $C_4H_6(NF_2)_4$     | 6.01  | 1.42              | 265 | 0.89  | BOF              |
|      | B                    | 10.20 |                   |     |       | CO               |
| VI   | $C_2(NO_2)_6$        | 53.80 | 1.437             | 287 | 0.976 | $N_2$            |
|      | $[C_4H_6(NF_2)_2]_x$ | 30.00 |                   |     |       | $H_2$            |
| VII  | $C_4H_4(NF_2)_4$     | 13.52 | 1.42              | 265 | 0.89  | BOF              |
|      | O                    | 9.71  |                   |     |       | CO               |
| VIII | $N_2H_5C(NO_2)_3$    | 56.77 | 1.42              | 265 | 0.89  | $H_2$            |
|      | $[C_4H_6(NF_2)_2]_x$ | 20.00 |                   |     |       | $N_2$            |
| IX   | $C_4H_6(NF_2)_4$     | 15.78 | 1.42              | 265 | 0.89  | BOF              |
|      | $N_2H_4(BH_3)_2$     | 25.71 |                   |     |       | +HCl             |
| X    | $NH_4ClO_4$          | 43.51 | 1.437             | 287 | 0.976 | +CO              |
|      | $[C_4H_6(NF_2)_2]_x$ | 15.00 |                   |     |       | $+H_2+N_2$       |
| XI   | $C_4H_6(NF_2)_4$     | 18.91 | 1.437             | 287 | 0.976 | BOF+             |
|      | $N_2H_4(BH_3)_2$     | 28.01 |                   |     |       | HCl+             |
| XII  | $NO_2ClO_4$          | 38.70 | 15.00             |     |       | CO+              |
|      | $[C_4H_6(NF_2)_2]_x$ | 15.00 |                   |     |       | $H_2+N_2$        |

What is claimed is:

1. A high-energy composite which on ignition burns at a controlled rate at a specific impulse in the range of 260 to 300 seconds, comprising 2 to 15 wt. percent boron, 5 to 25 wt. percent of a CNF<sub>2</sub> oxidizer selected from the group consisting of tetrakis (difluoramino) butane and tetrakis (difluoramino) tetrahydrofuran, 40 to 60 wt. percent of an oxygen oxidizer selected from the group consisting of nitronium perchlorate, hydrazinium nitroformate, hexanitroethane and ammonium perchlorate, and 5 to 30 wt. percent of a solid polymeric binder having the composition of polybutadiene (N<sub>2</sub>F<sub>4</sub>) adducts represented by the recurring unit composition [C<sub>4</sub>H<sub>6</sub>(NF<sub>2</sub>)<sub>y</sub>] in which y represents 1.3 to 2, NF<sub>2</sub> groups per recurring unit, the boron being in a 1:1 atomic ratio of fluorine in the composite to form BOF as a main combustion product.

2. A high-energy composite as defined in claim 1 in which the CNF<sub>2</sub> oxidizer is tetrakis (difluoramino) bu-

tane and the oxygen oxidizer is hexanitroethane.

3. A high-energy composite as defined in claim 1 in which the CNF<sub>2</sub> oxidizer is tetrakis (difluoramino) tet-

rahydrofuran and the oxygen oxidizer is hydrazinium nitroformate.

35 4. A high-energy composite as defined in claim 1 in which the CNF<sub>2</sub> oxidizer is tetrakis (difluoramino) butane and the oxygen oxidizer is ammonium perchlorate.

40 5. A high-energy composite which on ignition undergoes combustion to form BOF and CO as the main combustion products containing boron and oxygen present in the components of said composite, said composite containing 2 to 15 wt. percent boron, 5 to 25 wt. percent tetrakis (difluoramino) butane, 40 to 60 wt. percent nitronium perchlorate and 5 to 30 wt. percent polybutadiene (N<sub>2</sub>F<sub>4</sub>) adduct as solid binder, said binder containing 1.3 to 2 NF<sub>2</sub> groups per 4 carbon atoms, the boron in the composite being in a 1:1 atomic ratio to fluorine in the composite to form BOF as a main combustion product and the nitronium perchlorate supplying oxygen to form the BOF and CO.

\* \* \* \* \*